

H. F. Snyder, G. S. Snyder & W. N. Jones,

*Casting Journal Bearings.*

N<sup>o</sup> 85,341.

Patented Dec. 29, 1868.



Fig. 1.



Fig. 2.



Fig. 3.



Fig. 5.



Fig. 4.



Fig. 6.



Fig. 7.



Fig. 8.

Fig. 9.



Witnesses,  
G. S. Living  
W. C. Rullau.

Inventor;

H. F. Snyder G. S. Snyder  
W. N. Jones  
Per. *G. S. Snyder*  
Atty. *G. S. Snyder*



HENRY F. SNYDER, GEORGE S. SNYDER, AND WILLIAM N. JONES,  
OF WILLIAMSPORT, PENNSYLVANIA.

Letters Patent No. 85,341, dated December 29, 1868.

IMPROVEMENT IN CASTING BEARINGS FOR MACHINERY.

The Schedule referred to in these Letters Patent and making part of the same.

*To all whom it may concern:*

Be it known that we, HENRY F. SNYDER, GEORGE S. SNYDER, and WILLIAM N. JONES, of Williamsport, in the county of Lycoming, and in the State of Pennsylvania, have invented certain new and useful Improvements in the Manufacture of Boxes for Machine-Bearings; and we do hereby declare that the following is a full and exact description thereof.

Our boxes are mainly of iron, with a lining or bearing-surface of brass, cast therein in a novel manner. They may be cheaply produced, and combine the strength of iron with the frictional qualities of brass, and are highly durable and serviceable.

We will first describe what we consider the best means of carrying out our invention, and will afterwards designate the points which we believe to be new.

The accompanying drawings form a part of this specification.

Figure 1 is a side elevation of our boxes, complete. Figure 2 is a plan view of the same, represented as put together, before the projecting ends of the brass part are cut off.

Figure 3 is a cross-section through the centre of the same.

The remaining figures show the progress of the work at the earlier stages.

Figure 4 is a section through the mould before the iron is poured in. It represents the brass portion of the casting as having been previously cast in another mould, and fitted in its place in this mould, ready to have the iron poured in contact therewith, the brass being longer than the cavity for the iron.

Figure 5 represents a corresponding section of the mould after the iron has been poured and has commenced to impart its heat to the brass.

Figure 6 represents the same after the iron has heated the brass to about the same temperature as itself. At this stage the iron chills, or assumes a solid form, while the brass, by reason of its greater fusibility, assumes a liquid form, or melts. In this condition we turn up the entire mould and its contents upon one side.

Figure 7 shows the mould thus turned, and the metals cooling slowly, but the brass casting not yet shrunk materially.

Figure 8 shows the same after the brass has settled or sunk in cooling.

Figure 9 shows the entire box after it is completely cooled and removed from the mould.

Similar letters of reference indicate corresponding parts in all the figures.

A A are staves of brass, cast in any ordinary approved manner, and of length considerably greater than the bearing is intended to be when finished.

Now, having prepared a suitable mould in which to cast the iron part of our box, we introduce one of the staves of brass therein, and having properly closed the mould, we pour the iron so that it flows around the brass, and congeals there.

So soon as the iron is in contact with the brass, it commences to impart its heat thereto, and after a short time the brass stave A assumes a liquid form; in other words, it is melted by the heat received from the iron.

We take care, however, to pour the iron in at as low a temperature as it can be worked, and the iron cooled sufficiently further before the brass melts, so that by the time the brass has assumed a liquid condition the iron has assumed a solid condition.

The liquid brass ultimately cools, and assumes a solid form, and thus forms a lining imbedded in the iron.

The superfluous length given to the brass stave A allows for the shrinkage which comes in the cooling of the brass. We can place the stave in the mould so that both ends project, but this is not, in ordinary cases, necessary. We ordinarily place it with one end flush with the iron, and with the other end projecting, as indicated by C.

We judge, as nearly as possible, when the period has arrived when the brass will melt. At or a little before this period we turn the mould and its contents upon one side, so that the projecting end of the brass stave shall be uppermost. In this condition the melted brass settles by gravity into the cavity in the iron, and continues to fill it very tightly as the brass shrinks.

The final result is a casting of brass, filling the cavity in the iron, and adhering thereto with great strength, while the projection C is greatly contracted in its extent. In other words, the projection C of the brass, above the iron, forms a "sinking-head," which allows the brass to contract all that is required in the act of cooling, without forming any bubbles, or other faults.

We have experimented with this invention very extensively for several months, and have made, or caused to be made, in this manner, boxes varying from very small sizes up to the weight of five hundred pounds or more. These are in use in heavy mill-work in our vicinity, and are very highly approved.

We are aware that many efforts have before been made to combine iron with brass and other fusible metals, so as to obtain the surface of the softer metal with the strength of iron, but the previous attempts to cast them together have not come into use, by reason of the practical difficulties attending the operation.

Our method is perfectly successful. Not one cast-

ing has been lost since the workmen have become accustomed to the manipulation, so as to judge of the proper temperatures and periods.

We do not claim anything shown or described in the patent issued to Daniel Taylor, dated June 30, 1857; but having now fully described our invention,

What we claim as new, and for which we desire to secure Letters Patent, is as follows:

We claim the within-described mode of producing compound boxes, of iron and brass, united together,

forming the brass with a sinking-head projecting above the iron, so as to aid in compensating for the difference of contraction of the parts in cooling, substantially as herein set forth.

Witnesses:

T. C. ROGERS,  
H. D. HEISER.

H. F. SNYDER.  
G. S. SNYDER.  
W. N. JONES.